

June 21, 1955

D. C. GRESHAM

2,711,372

PHOTOMECHANICAL PROCESSES

Filed May 12, 1952

2 Sheets-Sheet 1

FIG. 1A



FIG. 1B



INVENTOR.  
DONALD CHARLES GRESHAM

BY

*Stevens, Davis, Miller & Kauper*

ATTORNEYS

June 21, 1955

D. C. GRESHAM

2,711,372

PHOTOMECHANICAL PROCESSES

Filed May 12, 1952

2 Sheets-Sheet 2

FIG. 2



INVENTOR.  
DONALD CHARLES GRESHAM

BY

*Stevens, Davis, Miller & Neese*  
ATTORNEYS

# United States Patent Office

2,711,372

Patented June 21, 1955

1

2,711,372

## PHOTOMECHANICAL PROCESSES

Donald Charles Gresham, London, England, assignor to  
McCorquodale & Company Limited, London, England,  
a British company

Application May 12, 1952, Serial No. 287,419

Claims priority, application Great Britain  
September 7, 1951

3 Claims. (Cl. 95—5)

This invention relates to photomechanical processes and particularly to the production of records of discontinuous tone subjects and is an improvement in or modification of my Patent No. 2,704,252 filed 15th January, 1951.

In Patent No. 2,704,252 I have described inter alia a new method of producing positives directly from originals by a reversal technique, which method comprises exposing a photographic plate or film to light from an original subject, developing to silver the latent image obtained, thereby producing a negative image in silver, producing a coloured image in situ therewith and bleaching the said silver image, exposing the said plate or film to light incident on the same side thereof as the original exposure, the said light being of a colour to which the photographic emulsion is sensitive but which is absorbed by the said coloured image, redeveloping the said plate or film, fixing the plate or film to remove any residual silver halide, and removing the coloured image. The coloured image may be formed by dye-toning or mordanting but in the preferred form of the invention the first development is effected by means of an aromatic primary amino compound in the presence of a colour former which couples with the oxidation products of the developer to form a dyestuff image.

By the said process a positive image in silver is directly obtained. Owing to the fact that the dyestuff negative image absorbs the re-exposure light the silver halide lying below the dyestuff image is not re-exposed. Accordingly it is not necessary to go to the length of full first exposure and commercial variations in emulsion thickness have no effect on the result obtained. Generally speaking it is sufficient to use photographic plates or films which are not optically sensitised, i. e. which have only their natural sensitivity to blue light. With such plates and films it is preferred that the colour former should be one which yields a yellow or yellow-orange image. The colour former may be included in the original photographic emulsion or may be included in the developer used for the first development only. Generally speaking the second development will be effected by means of a developer which does not, in the presence of a colour former, yield a dyestuff image, but where the colour former is contained in the emulsion the selection as second developer of an aromatic primary amino developing agent, which will yield with such colour former a dye image in situ with the silver image is not excluded since the positive dye image thus formed will be removed at the same time as the negative dye image so that the final product will be unchanged.

A wide range of colour formers is described in the literature and examples of colour formers suitable for the present invention may be selected from the list of yellow-orange colour formers set out in the British Journal of Photography, volume 85, p. 648.

It is, of course, important that the agent selected for use in bleaching the initially formed negative silver image should be one which does not adversely affect the residual silver halide or the dyestuff image. A suitable bleach-

2

ing agent consists of an aqueous solution of potassium ferricyanide and potassium bromide.

In order that no image should be developed in the "negative area" of the plate or film during the second development stage it is important that all the silver halide rendered developable in the first exposure should be developed in the first development. This can usually be achieved by prolonging the first development step, but, as an alternative the first development can be completed by treating the plate or film in a vigorous developer, e. g. a metol-hydroquinone type of developer. The developer used for the second development stage, producing the positive image, is preferably one giving a high contrast image and caustic soda-hydroquinone developers have been found very useful. It is advantageous to include a small quantity of an anti-fogging agent in this second developer, e. g. benzotriazole or any other of the well known heterocyclic compounds having anti-fogging action when included in developers.

The removal of the dye image is usually effected as a final stage in the preparation of the screen positive. Generally speaking, the quinone-imine or azomethine dyes produced by colour developers, using colour formers of relatively simple structure, are soluble in common organic solvents and one convenient method of removing the dye image therefore is to bathe the plate or film in an organic solvent medium for the dyestuff. A suitable medium for many colour-formed dyestuffs is a mixture of methyl alcohol, acetone and glacial acetic acid.

As stated in application Serial No. 206,120 the foregoing method is especially suitable for the reproduction of line originals. It affords results as good as are obtained by the usual negative-positive process and has the additional advantage that only a normal negative exposure is required instead of a greatly increased exposure as in the conventional reversal process. Moreover the product is laterally correct for litho printing and so obviates the use of a prism on the camera.

In the drawing:

Fig. 1(A) is a diagrammatical illustration showing the effect obtained by the process just described.

Fig. 1(B) is a diagrammatical illustration illustrating the process of the present invention.

Fig. 2 is a flow sheet illustrating the steps in the process of the present invention.

The effect obtained by the aforesaid process is diagrammatically illustrated in the accompanying Fig. 1(A) of the drawings. It will be observed that the negative image is formed in dye and silver and the latter is bleached (i. e., halogenized). The areas between the discontinuous negative areas are exposed by the second exposure and the silver halide lying below the said negative areas is not re-exposed. It will further be observed from the drawing that the result is independent of emulsion thickness. The emulsion has been illustrated with an exaggerated variation in thickness but the areas of the discontinuous image obtained is independent of this variation. The ordinary reversal process, however, in which the whole of the silver halide which was unused in the first exposure is exposed in the second exposure is essentially dependent on emulsion thickness variations. The line AA on this drawing illustrates diagrammatically the effect of a uniform second exposure. It will be understood that the drawing is purely diagrammatic and that the depth of the image areas represents not so much their physical depth but their effective density.

It has been found however that where the process is applied to the reproduction of line originals of such character as dry-point etchings, where the original contrast is very low and moreover the finest lines are usually of very low density and the closely hatched shadow areas tend to be more or less blocked-up, the quality of the

reproduction obtained is still not all that could be desired. This is also the case where the original is itself a screen image.

Such originals may generally be described as "fine detail discontinuous tone" originals. According to the present invention a method of producing positives directly from fine detail discontinuous tone originals by a reversal technique comprises exposing a photographic plate or film to light from such original subject, developing to silver the latent image obtained, thereby producing an image in silver, producing a coloured image in situ therewith and bleaching the said silver image, exposing the said plate or film to light incident on the same side thereof as the original exposure, the said light being of a colour to which the photographic emulsion is sensitive but which is absorbed by the said coloured image, the second exposure being effected at least partially to light from the original subject, redeveloping the said plate or film, fixing the plate or film to remove any residual silver halide and removing the coloured image. Since the highlights of the original subject reflect most light and the shadows least light the effective re-exposure of the plate or film is greatest in the highlights and least in the shadows, which results in a correction of the gradation while providing the correct tonal range.

In practice it has been found that the relative intensities of the highlights and shadows of the original subject are usually such that, if the whole re-exposure is effected to the original subject an over-correction results. Accordingly in the preferred form of the invention, part of the re-exposure is effected to the original subject, sufficient to effect the desired tonal correction, and the remainder of the re-exposure is effected to uniform light. The optimum ratio of these exposures depends on the photographic material and the method of plate making employed but is generally found to be of the order of 15 to 30:1.

The effect obtained is diagrammatically illustrated in Fig. 1(B) of the drawings. This figure is similar to Fig. 1(A) but the line BB is shown drawn at an angle to represent the effect of a second exposure which is modulated image wise by the original. The effect of this is greatest in the regions corresponding to those regions of the original which have the least area of black detail and, as shown, allows the negative to be made with sufficient exposure to record detail adequately in closely hatched areas of the original. Such exposure would normally be excessive for adequate recording of the fine detail in open areas of the original particularly if, as is often the case, such detail has low density.

In carrying out this form of the invention the plate or film, after first development, is replaced, either in wet or dry condition, in the process camera and registered in its original position so that the second recorded image is exactly in register with the first recorded image. An exposure sufficient to effect the desired tone-correction is then effected and thereafter the original is covered with a sheet of white reflecting material and the exposure continued until the required total re-exposure is reached. Both parts of the re-exposure are, of course, effected via an appropriate filter selected to transmit only light of wavebands absorbed by the negative dye image (which may be associated with the re-halogenised silver).

A flow sheet of this method is illustrated in Fig. 2. Referring to this drawing a fine line original 11 is copied in the camera (illustrated as lens 12) on to a photographic element 13A. The element 13A is color developed, washed, treated to bleach the silver image, washed, drained, and (now identified as 13B) replaced in the camera in its original position. The second exposure is made partially to original 11 and partly to a white card 14. The element 13B is then processed to develop a silver image, to remove residual silver halide and bleach negative silver, washed and treated to remove the dye image. This gives the final product 13C which

carries a silver fine line position which records faithfully both fine isolated black detail and closely hatched dark areas of the original.

The following example will serve to illustrate the invention.

#### Example

A camera with a process lens of 18 inch focal length was used and the illumination consisted of four 30 amp. open-arc lamps at 3½ feet from the centre of the copy board.

A dry-point etching was set up on the camera as the original. The scale of reproduction was  $\times 0.7$ , requiring a camera extension of 740 mm.

1. A Kodak B5 "Process Slow" plate was placed in the camera and an exposure of 22 seconds was given to the original through a tri-colour blue filter (Wratten 49— the word "Wratten" being a registered trade-mark) at a lens aperture of 11.5 mm.

2. The plate was developed for 7½ minutes at 65° F. in a yellow-forming colour developer constituted of equal parts of the following solutions A and B.

|                                                                      |    |      |
|----------------------------------------------------------------------|----|------|
| A. N.N-diethyl-p-phenylene diamine, sulphur dioxide reaction product | g  | 4.5  |
| Sodium sulphite (anhydrous)                                          | g  | 18.5 |
| Potassium bromide                                                    | g  | 4    |
| Water to make 2250 cc.                                               |    |      |
| B. Acetone                                                           | cc | 200  |
| 2.5-dichloracetoneacetanilide                                        | g  | 20   |
| Sodium hydroxide                                                     | g  | 14   |
| Sodium carbonate (anhydrous)                                         | g  | 132  |
| Water to make 2250 cc.                                               |    |      |

3. The plate was washed for 2 minutes.

4. The plate was bleached for 5 minutes in a solution of 50 g. potassium ferricyanide and 50 g. potassium bromide in a litre of water.

5. The plate was washed for 10 minutes.

6. The plate was replaced in the camera in precisely the same position as it occupied for the first exposure.

7. The plate was re-exposed to the original subject, without a filter for 210 seconds, the lens being at full aperture (46 mm.). The original subject was then covered with white paper and a further exposure given of 10 seconds at a lens aperture of 27 mm.

8. The plate was then developed for 4 minutes at 65° F. in a developer made up of equal parts of the following solutions A, B and C.

|                                 |    |    |
|---------------------------------|----|----|
| A. Hydroquinone                 | g  | 38 |
| Potassium metabisulphite        | g  | 38 |
| Potassium bromide               | g  | 19 |
| Water to make 2 litres.         |    |    |
| B. Potassium hydroxide          | g  | 75 |
| Water to make 2 litres.         |    |    |
| C. 1% solution of benzotriazole | cc | 45 |
| Water to make 2 litres.         |    |    |

9. The plate was fixed in an acid hardening fixing bath.

10. The plate was washed, bathed in a mixture of 900 cc. industrial spirit and 100 cc. glacial acetic acid to dissolve away the colour-formed dye image, and dried.

The resulting line positive was printed down on metal and gave excellent reproductions of the original when printed by the photo litho off-set process.

The conditions of first development in the color development given in the foregoing example will yield a gamma value of about 3.0 on an average batch of the sensitive material specified but on any batch of the material the gamma value will be at least approximately 2.5 as will be appreciated by those skilled in the art. The conditions of second development given in the example will yield a gamma value of about 5.0 on an average batch of the sensitive material specified but on a batch of the material the gamma value will be at least approximately 4.0.

75 In accordance with a further aspect of the present

invention line originals are reproduced by printing down in register a line positive of the original made by the process of the invention and a screen positive of the original made by the process of application Serial No. 206,120. Thus for example a line positive may be made by the process set out in the foregoing example and a screen positive of the same subject may be made by the process of Example 2 of application Serial No. 206,120. By printing these positives down onto metal and printing the line positive record in black and the screen positive record in grey, a reproduction of the original subject of remarkably high fidelity is obtained.

It is sometimes desirable to make a screen positive by enlargement from small screen images. This is particularly useful for posters which may be larger than the largest screen available but where a coarse screen image resulting from the enlargement is not a disadvantage. The usual procedure is to make a normal screen negative and to rephotograph the trans-illuminated negative in the camera without the screen and at the required magnification. This usually results in a screen positive with excessive contrast and poor tonal gradation. The process of the present invention provides a definite solution to this problem. The preferred method is as follows:

A screen positive is made from a continuous tone original, retouched and proofed. The screen positive is preferably made by the method described in application Serial No. 206,120 but any screen positive which gives a satisfactory proof can be used. The screen positive is set up in the transparency holder of the camera and is photographed on a photographic element of inherently high contrast characteristics, at the required magnification. The photographic element is developed in a colour developer and the silver is rehalogenised in a ferricyanide-bromide bath. The photographic element is then replaced in the camera in the position it occupied for the first exposure and is given an exposure to the original screen positive followed by a uniform exposure. A very small amount of diffusion may usefully be introduced during the exposure to the original screen positive, for instance by placing a sheet of matt plastic in contact with the camera side of the original screen positive. These exposures must be by light of a colour to which the plate is sensitive but to which the dye image has high density. Finally the photographic element is developed in a high contrast developer, fixed and the dye is removed. By suitably adjusting the ratio of uniform exposure to image-wise exposure it is possible to obtain an exact reproduction of the tone value of the original screen positive and, since the original positive has been proofed, the result which will be obtained from the enlarged positive may in this way again be accurately predicted. The actual ratio of exposures required depend on the apparatus in use but once they have been determined they remain constant. The method may be applied to multicolour reproduction, e. g. four-colour reproduction, by repeating the procedure for colour-separation screen positives made from the original.

It will be noted that in the foregoing example the photographic material specified has an emulsion with "high contrast" and when this expression is used in the appended claims it has reference to one of the many commercially available materials made primarily for the production of linear screen records. At the present time these fall into classes which I define as follows: (a) Materials which, when exposed to white light and developed for 3 minutes at 68° F. in Kodak developer D11, yield a gamma value of at least 3.5; (b) materials of the "Kodalith" type which have silver chloride emulsions and when developed in special developers containing formaldehyde or reaction products of formaldehyde yield a gamma value of at least 4.0.

When I refer to a gamma value of a dye image I refer to a figure derived by developing a step wedge on the material to be used in the color developer to be used,

fixing out the undeveloped silver halide in a fixing bath which does not appreciably affect the dye image, bleaching the silver image in the bleaching bath to be used, measuring the densities of the wedge steps through a filter of complementary color to the dye image, plotting these densities against the logarithms of the exposures which produced them and deriving the gradient value from the curve in the usual way.

I claim:

1. A method of producing positives directly from fine detail discontinuous tone originals by a reversal technique which method comprises exposing a photographic element having an emulsion of high contrast to light from such original subject, developing the fine line latent image thus obtained with an aromatic primary amino developing agent in the presence of a color coupler which combines with the oxidation products of such developer to produce a dye image, thereby producing a negative image made up of areas of developed silver with a dye image in situ therewith, said development being such as to produce a dye image with a gamma value of at least approximately 2.5, bleaching the said silver image, exposing the unexposed areas of the said element to light incident on the same side thereof as the original exposure, the said light being of a color to which the photographic emulsion is sensitive and being of such color and intensity that the light is substantially completely absorbed by the said colored image, the second exposure being effected at least partially to light from the original subject, redeveloping the said element to a gamma of at least approximately 4.0 in a developer which will not redevelop any rehalogenized silver negative image which may be present, fixing the element to remove the residual silver halide remaining below the negative image which has been optically screened from the second exposure, any silver halide remaining below the positive image and any rehalogenized silver of the negative image which may be present, and then removing the negative dye image.

2. A method of producing positives directly from fine line originals by a reversal technique which method comprises exposing a photographic element having an emulsion of high contrast to light from such original subject, developing the fine line latent image thus obtained with an aromatic primary amino developing agent in the presence of a color coupler which combines with the oxidation products of such developer to produce a dye image, thereby producing a negative image made up of areas of developed silver with a dye image in situ therewith, said development being such as to produce a dye image with a gamma value of at least approximately 2.5, bleaching the said silver image, exposing the unexposed areas of the said element to light incident on the same side thereof as the original exposure, the said light being of a color to which the photographic emulsion is sensitive and being of such color and intensity that the light is substantially completely absorbed by the said colored image, the second exposure being effected at least partially to light from the original subject, redeveloping the said element to a gamma of at least approximately 4.0 in a developer which will not redevelop any rehalogenized silver negative image which may be present, fixing the element to remove any residual silver halide and removing the colored image.

3. A method of producing positives directly from fine line originals by a reversal technique which method comprises exposing a photographic element having an emulsion of high contrast to light from such original subject, developing the fine line latent image thus obtained with an aromatic primary amino developing agent in the presence of a color coupler which combines with the oxidation products of such developer to produce a dye image, thereby producing a negative image made up of areas of developed silver with a dye image in situ therewith, said development being such as to produce a dye image with a gamma value of at least approximately 2.5, bleaching the said silver image, exposing the unexposed areas of

said element to light incident on the same side thereof as the original exposure, the said light being of a color to which the photographic emulsion is sensitive and being of such color and intensity that the light is substantially completely absorbed by the said colored image, the second exposure being effected partly to light from the original subject and partly to uniform light, the ratio of these parts being 15 to 30:1, redeveloping the said element to a gamma value of at least approximately 4.0 in a developer which will not redevelop any rehalogenized silver negative image which may be present, fixing the element to remove any residual silver halide and removing the colored image.

5  
10

## References Cited in the file of this patent

## UNITED STATES PATENTS

|           |                |               |
|-----------|----------------|---------------|
| 2,165,407 | Murray         | July 11, 1939 |
| 2,182,814 | Marasco        | Dec. 12, 1939 |
| 2,327,822 | Russell et al. | Aug. 24, 1943 |

## FOREIGN PATENTS

|         |         |              |
|---------|---------|--------------|
| 593,839 | Germany | Mar. 6, 1934 |
|---------|---------|--------------|

## OTHER REFERENCES

Process Engraver's Monthly, February 1947, page 50;  
August 1948, pp. 236-237; September 1948, pp. 287-288.